

## UNITED STATES PATENT OFFICE

WILLIAM HOWARD WRIGHT, OF SCHENECTADY, NEW YORK, ASSIGNOR TO  
SCHENECTADY VARNISH COMPANY, OF SCHENECTADY, NEW YORK, A CORPORA-  
TION OF NEW YORK

## COMPOSITION

No Drawing.

Application filed October 13, 1927. Serial No. 228,035.

The present invention relates to an oil proofing composition, and while particularly adapted for impregnating transformer coils, may, nevertheless, be used in a variety of instances and applications where it is desired to render a particular substance greaseproof and waterproof.

In the case of transformer coils where the conductor is usually covered with an insulating material, such as paper, vegetable or animal fabric, arcing frequently results between different coils, due to corrosion of the insulation, and difference in potential between the coils. While the oil in which the 10 transformers are immersed is a cooling and insulating medium, nevertheless, such oil has frequently been found to contain materials rendering it conductive or to have had its chemical constitution so changed that it will 15 allow an arc to jump from one transformer coil to another. Where, as stated, the insulation about the conductors has decayed and there exists a difference in potential between the one or more adjacent transformers, the 20 oil may be of such character as to permit of arcing, and thus destroy the efficiency of the 25 transformers.

The difficulty heretofore has been to find a material which would not be dissolved by 30 mineral oils in oil cooled transformers. As is well known, these transformers run at a considerable temperature rise, and it is essential that the insulation of the coils be insoluble in the hot mineral oil. The proper 35 cooling of the transformers depends on the rapidity of circulating of the oil in the transformer tank surrounding the coils. Where the insulation is soluble, the oil becomes heavy 40 and the circulation of the oil impeded. Hence the cooling of the coils is not as efficiently done as when the oil is thinner, and the temperature rise of the machine consequently higher and its electrical capacity 45 lower.

To this end, therefore, my invention has 50 in mind the protection of the di-electric or insulator surrounding the conductor from the corrosive action of the oil, and thus assist in maintaining the conductor always

properly insulated so as to prevent the possibility of arcing.

A very important object of this invention is therefore the provision of an oilproof coating composition which is not only insulating but which is moreover insoluble in the hot or cold oil surrounding the transformer. In this manner, the circulating efficiency of the oil is increased and no objectionable chemical compounds are formed.

A further object of the invention is to provide a composition of this character which may be prepared in liquid form, or prepared in liquid form, permitted to solidify and then subsequently rendered fluid for impregnation and coating purposes.

The invention has, moreover, in mind the production of a plastic which may be suitably shaped or moulded and also rolled, and when cooled is a hard solid substance of nice 70 appearance, non-conductive and waterproof.

The composition of the present invention comprises preferably a resin such as rosin, colophony or abietic acid. I have found, however, that resins containing gums, etheral oils and other important constituents may be employed, and in fact any resinous material may be utilized in accordance with requirements and the product desired.

With the resin, I preferably mix or combine a natural gum which is a species of Xanthorrhœa. One of such gums which I have used is accroides or acaroids of which there is an abundant and cheap supply obtainable from Australia.

There are two kinds of gum accroides both characterized by being esters of paracoumaric acid.

Other species of Xanthorrhœa may be employed in accordance with the product desired, but I will here set forth the red and yellow gum accroides.

Red accroides comprises paracoumaric acid ( $C_9H_8O_3$ ) 1%; benzoic acid in traces and paracoumaric acid 2%, both in combination with erythrosinotannol ( $C_{10}H_{20}O_9OH$ ); paraoxybenzaldehyde .6%. The bulk, 85%, consists of the erythrosinotannol ester of paracoumaric acid. The absence of cinnamic 100

acid distinguishes this resin from yellow acaroid.

The yellow acaroids comprise free para-coumaric acid ( $C_9H_8O_3$ ) 4%; free cinnamic acid 5%; combined paracoumaric acid 7%

5 and combined cinnamic acid 6%. Both acids form esters with xanthroresinotannol



10 producing chiefly the corresponding ester of paracoumaric acid which forms the main constituent of this resin.

Also there are probably present styracin ( $C_{18}H_{16}O_2$ ), cinnamic phenylpropyl ester, 15 paraoxybenzaldehyde, and possibly vanillin.

20 To this mixture may be added vegetable, animal and mineral oils, or other resins, both natural and synthetic, for instance, the product known commercially as paracumaron.

25 However, the resin and gum are the fundamental ingredients, and the other substances may or may not be added, as desired.

30 The proportion of the ingredients is determined by the melting point of the finished compound desired. This melting point varies for most purposes from 100° C. to 150° C. in accordance with the particular type of coil or conductor to be treated.

35 The difference in the melting points may be easily obtained by using a greater or less amount of each ingredient in the mixture, it being found that a composition consisting of equal parts of the two materials will suffice for a large number of cases.

40 It has been found useful in some instances to add to the mixture other materials for instance, castor oil or fatty acids in the nature of stearic acid and other resins of both natural and synthetic character. These sub-

45 stances may be added singly to a mixture of rosin and gum accroides or in some cases both stearic acid and castor oil may be used, or these two ingredients together with other resins may be employed. Also either stearic acid or castor oil may be employed in conjunction with such other resins in accordance with requirements of a particular case.

50 The castor oil and other oils for instance, serve to reduce the brittleness of the resin and accroides composition, while stearic acid acts in some cases as a flux to give a better combination of the two main ingredients with or without the castor oil or other resins.

55 The use of resins natural or synthetic, for example, paracumaron, is useful at times for varying the melting point of the composition and for determining its solubility in connection with various types of transformer oils.

60 For example the mixture may comprise: Rosin, gum accroides, castor oil. Rosin, gum accroides, stearic acid. Rosin, gum accroides, castor oil, stearic acid.

Rosin, gum accroides, resins (natural or synthetic).

Rosin, gum accroides, stearic acid, resins (natural or synthetic).

Rosin, gum accroides, castor oil, resins 70 (natural or synthetic).

Rosin, gum accroides, stearic acid, castor oil, resins (natural or synthetic).

As previously stated, for a great number of instances, a plain mixture of gum accroides and rosin in equal parts will suffice 75 and the proportions of these constituents may be varied to change the melting point. The melting point may be changed for example by adding a greater or smaller amount 80 of rosin.

Where a single one of the ingredients above noted is employed, they may comprise up to approximately ten per cent (10%) of the mixture.

85 For instance, in the use of castor oil or resins ten per cent (10%) of the mixture has been found sufficient. In the case of stearic acid, the amount found necessary for the best result is approximately five per cent 90 (5%). Where the ingredients are employed together, their total proportion should be substantially ten per cent (10%) of the mixture.

95 Of course, a quantity more or less may be useful in accordance with the character of rosin, and the nature of the gum, and the percentage of proportions here recited are those which have been found experimentally and practically satisfactory with a wide 100 range of ingredients and applications.

105 In preparing my improved oil-proof and waterproof composition, the gum accroides and rosin together with the addition ingredients, if employed, may be melted together or separately, and mixed in fluid condition to the proper consistency, and the fluid strained and permitted to cool into a hard solid compound having a melting point from 100° C. to 150° C., more or less. By having 110 the product in solid form, it may be easily transported and employed as desired.

115 In treating transformer coils or for other impregnation purposes, a series of tanks of suitable size are employed. In one of the tanks, the composition of the present invention is placed and melted to a fluid condition, say at a temperature of approximately 325° F. The other tank receives the coils and is preferably provided with means for exhausting air therefrom, being in the nature of a closed container. After the air has been exhausted, the coil contained in the chamber is heated to expel any moisture. Thereafter, the melted material in the other tank is 120 passed into the chamber containing the article to be treated, and the article immersed in the treating substance.

125 Pressure is then applied in the closed chamber containing the coil or other article 130

immersed in the composition of my invention, and such pressure is maintained for a sufficient time to force the compound into the di-electric covering of the coils or article 5 to be impregnated. There results a hard coating thoroughly oilproof and insoluble in the hot or cold oil surrounding the transformer.

As previously stated, the ingredients of my composition are preferably melted together until the proper consistency or degree of plasticity is reached, such that a uniform product may be obtained, and thereafter permitted to cool into solid form.

15 This is the finished article which is utilized in the impregnating process just described.

My invention is obviously useful for a great variety of applications where a grease-proof or waterproof impregnation compound is desirable. For example, the ingredients herein recited may be dissolved in alcohol, petroleum, naphtha, menthanol and a 20 variety of other solvents, or two or more of these solvents may be used together.

25 This solution so obtained may be applied to a surface to be treated by means of spraying, brushing, dipping or other mechanical process, and it has been found under such circumstances that a hard insoluble impregnation and protective coating is produced.

30 It will be understood, of course, that a great variety of vegetables, animal and mineral oils other than castor oil may be used as the addition ingredients of my invention, as well as resins of various types, both natural 35 and synthetic.

35 In referring to the use of paracumaron, it will be understood that I have in mind a resin having this commercial trade name, or a resin 40 having the formula  $C_8H_6O$ . I also have in mind the use of commercial cumaron which is a mixture of paracumaron and para indene. These materials may be used in combination with a resin or with fatty acids such 45 as castor oil and stearic acid, as previously described. It will be understood, however, that the composition so obtained is not the full equivalent of the natural gum accroides and resin, although it may be used for the 50 same purpose. I have also found that paracumaric acid combined with a resin has excellent oil proofing qualities, but the results are not as good as a composition of rosin and gum accroides, as described.

55 My composition is a non-conductor, and in some cases may be employed solely as the insulating material or impregnating agent.

In other cases, as for example, electrical applications, it may be used to impregnate the 60 di-electric or insulator and to afford not only a greater insulation, but a protection to the first coating, which will prevent its decay or corrosion, due to the action of either the atmosphere or as in the case of transformer 65 coils, the action of the oil in which such coils

are usually immersed, tending to dissolve it. It must, moreover, be understood, that since I obtain a solid product, this product is available in its solid form for a great variety of purposes where an insulating or waterproof 70 material is desirable, and the solid product may be shaped, if preferred, and sawed or cut to any desired form, for example, while the composition is cooling after a proper mixture is obtained, such cooling may be accomplished in a suitable mold, or the material 75 may be rolled into sheets.

The present invention is not limited, therefore, to a coating or impregnating compound, although the composition is especially useful in this connection, since, obviously, it may be used in its solid form for an innumerable number of purposes, meeting requirements for which it is characteristically useful.

80 It will be understood that in some cases the materials may be placed in a tank adjacent to the article to be treated, and there melted and mixed to the desired consistency, and then propelled or transported to the treating chamber. This step would be desirable in some operations, and would eliminate the necessity of awaiting the cooling of the mixture to solid form.

85 In making a plastic composition, which can be rolled into sheets and cut to suitable sizes and shapes or moulded to various shapes, it may be desirable to add a hardening agent, and for this purpose any well known material may be used. Of course, heat and pressure either together or separately may be 90 employed, depending, of course, upon the 95 nature of the composition.

100 I claim:

1. In the art of treating electrical coils having a covering and adapted to be immersed in a cooling medium such as oil, the 105 step which comprises impregnating the covering of such coils with a composition insoluble in the oil comprising an accaroid resin.

2. In the art of treating electrical coils having a covering and adapted to be immersed in a cooling medium such as oil, the step which comprises impregnating and coating the covering with a composition insoluble in 110 the oil comprising an accaroid resin, the said composition forming a hard coating about the coils.

3. In the art of treating electrical coils having a covering and adapted to be immersed in a cooling medium such as oil, the step which comprises impregnating the covering with a composition insoluble in the oil comprising an accaroid resin and a pure resin.

4. In the art of treating electrical coils having a covering and adapted to be immersed in a cooling medium such as oil, the step which comprises impregnating and coating such covering with a composition insoluble in the oil comprising an accaroid resin 120

and a pure resin, the said composition forming a hard coating about the coils.

5. In the art of treating electrical coils having a covering and adapted to be immersed in a cooling medium such as oil, the step which comprises impregnating such covering with an insulating composition insoluble in oil comprising an accaroid resin, rosin and one or more agents in the nature of castor

10 oil, stearic acid, and another resin.

6. In the art of treating electrical coils having a covering and adapted to be immersed in a cooling medium such as oil, the step which comprises impregnating and coating such covering with an insulating composition insoluble in the oil comprising an accaroid resin, rosin and one or more addition agents in the nature of castor oil, stearic acid and another resin, the said composition

20 forming a hard coating about the coils.

7. In the art of treating electrical coils having a covering and adapted to be immersed in a cooling medium such as oil, the step which comprises covering such coils with an

25 insulating composition comprising an accaroid resin and a plasticizer.

8. In the art of treating electrical coils having a covering and adapted to be immersed in a cooling medium such as oil, the

30 step which comprises covering such coils with an insulating composition comprising an accaroid resin, rosin and a plasticizer.

9. In the art of treating electrical coils having a covering and adapted to be immersed

35 in a cooling medium such as oil, the step

which comprises coating such coils with an insulating composition comprising an accaroid resin, rosin and a plasticizer and flux.

10. An electrical coil impregnated and

40 coated with an oil proof and water proof

composition comprising an accaroid resin

and forming an insoluble coating about the

coil.

In testimony whereof I have hereunto set

45 my hand.

WILLIAM H. WRIGHT.